

## UNITED STATES PATENT OFFICE

2,456,471

## PROCESS AND PASTE FOR PRINTING FABRICS MADE OF CELLULOSE, SUCH AS TEXTILE FABRICS, PAPER AND THE LIKE, WITH CHROMIUM MORDANT DYESTUFFS

Ernst Tschan, Basel, Switzerland, assignor to Durand &amp; Huguenin A. G., Basel, Switzerland, a Swiss firm,

No Drawing. Application March 15, 1945, Serial No. 583,007. In Switzerland February 17, 1944.

Section 1, Public Law 690, August 8, 1946  
Patent expires February 17, 1964

14 Claims. (Cl. 8—72)

## 1

As known, the chromium mordant dyestuff had formerly always to be fixed by a prolonged steaming. In order to obtain a complete formation of the chromium lake, a steaming of at least 45 minutes was required. After the knowledge of readily fixable dyestuffs, such as vat dyestuffs, ester salts of leuco vat dyestuffs and naphthol dyestuffs, the necessity of a long steaming has been felt as a drawback by the consumers. Consequently the application of chromium mordant dyestuffs has retrograded considerably.

However, the above mentioned drawback was overcome to some extent, inasmuch as the formation of the lake could be accelerated a good deal by the addition to the printing pastes of carboxylic acid amides, such as urea, formamide or acetamide (see Melland Textilberichte 1933, page 412 and 1934, page 362: "Ueber einige Fortschritte in der Anwendung der Chromfarbstoffe" by G. von Niederhäusern, and French Patent No. 865067).

It is further known, that the chromium mordant dyestuffs can be fixed on cellulose fibres by a steaming of 8 minutes with the assistance of sodium chromate in presence of a reducing agent (see Recipes, Durand & Huguenin S. A., part II, second edition, pages 39 et seq.).

These different processes already represented a considerable technical improvement compared with former long steaming processes. They facilitated considerably the practical application of the chrome mordant dyestuffs. Thus a great number of chromium mordant dyestuffs could now well be fixed on cellulose fibres by a steaming of 5-8 minutes in a Mather-Platt ager. But, when working according to the above mentioned processes with a short steaming duration, it was impossible to obtain a yield as good as that obtained by the application of the former processes with a long steaming. Nevertheless the loss of dyestuff—wherever it occurred—was put up with, when considering the great acceleration of the working method resulting by applying these new processes and the economy resulting therefrom.

It has now been found that the formation of the chromium mordant dyestuff lake, i. e. the fixation of the dyestuff on the printed fabrics can considerably be accelerated by using printing pastes containing beside the dyestuff, the thickener and possibly other usual additions, such as: formic acid, acetic acid and the like; a carboxylic

acid amide, an alkali chromate or bichromate as mordant agent, furthermore a soluble salt of an acid deriving from an oxygen compound of sulphur and possessing reducing properties, a substance capable of splitting off a strong acid in the heat, as well as, if convenient, an aromatic compound, such as a polyhydroxy compound or polyketone respectively, which is capable of performing the reversible reaction: quinone $\leftrightarrow$ hydroquinone and which may be present in the form of quinone as well as in the form of hydroquinone and finally containing  $\omega,\omega'$ -dihydroxydiethylsulphide; by printing such printing pastes on the fabrics and forming the chromium lake, without any steaming, by a simple drying and if desired hanging.

If for instance a fabric consisting of cellulose fibres is printed with such a printing paste, dried and left hanging or lying for 48 hours at room temperature, then rinsed and, as usual for chromium mordant dyestuffs, subsequently soaped, rinsed again and dried, there are obtained well fixed chromium mordant dyestuff prints, without necessitating a steaming operation for the formation of the chromium lake.

Hitherto it was impossible to obtain chromium mordant dyestuff prints meeting practical requirements without any steaming. The elimination of the steaming process means an important improvement and for many works a considerable simplification and facilitation of the working process. Moreover, the new process allows the use of chromium mordant dyestuffs in all those cases where steaming is impossible, such as, for instance, for printing paper, paper hangings, woven paper and similar fabrics. In this case, the printed paper is dried on a drying cylinder and left lying, whereby the colours are themselves normally fixed. The prints thus obtained are fast to washing and rubbing.

It is understood that chromium mordant dyestuff printing pastes obtained according to the above disclosures may also be fixed by steaming. In this case, a very short steaming of 2 minutes will be sufficient, this being a lapse of time which heretofore would not have been sufficient for the fixation. When steaming is applied, the above mentioned aromatic polyhydroxy compounds or aromatic polyketones respectively, as well as, in

## 2

most of the cases, also the  $\omega:\omega'$ -dihydroxydiethylsulphide may be dispensed with in the printing pastes. Also this variation of the process involves a considerable technical improvement compared with the methods known up to now, inasmuch as thus a yield is obtained which could not be attained even by a three-fold steaming duration.

For carrying out the process, sodium or ammonium chromate may be used as mordant agent. Also bichromates will give pretty good results; however, in the latter case, the stability of the printing pastes is poor. As soluble salts of acids deriving from oxygen compounds of sulphur and possessing reducing properties may be enumerated: hydrosulphites, sulphites, thiosulphates, whereby according to the dyestuff used the most suitable one of the salts will advantageously be selected.

As acid yielding substances suitable for the process there may be used the salts of a volatile inorganic or organic base with a strong inorganic or organic acid, the latter being not allowed to disturb the formation of the dyestuff chromium lake. As examples may be mentioned: ammonium sulphocyanate, ammonium chloride, ammonium sulphate, ammonium nitrate, etc.

As aromatic polyhydroxy compounds which are converted into quinones by oxidation, use may be made of for instance: hydroquinone, pyrocatechine, resorcinol, pyrogallol, phloroglucine, hydroxyhydroquinone. Suitable aromatic polyketones which are transformed into a hydroquinone by reduction are:  $\alpha$ -naphthoquinone, anthraquinone, quinizarine and the like, as well as the sulphonic acids of the substances of both these groups.

All the above mentioned additional products may be added to the printing paste or the latter may be prepared in two separate portions, one portion containing the dyestuff, the accelerator,  $\omega:\omega'$ -dihydroxydiethylsulphide, the thickener and the acid yielding substance, moreover the salt of an acid deriving from an oxygen compound of sulphur and possessing reducing properties, the other one containing the chromium mordant, the aromatic compound, i. e. the polyhydroxy compound or the polyketone and also the thickener. The two portions will subsequently be mixed up together before printing.

The new process is illustrated by the following examples; without being limited thereto. The parts are by weight.

#### Example 1

The following printing colour is printed on cotton or staple fibres:

|                                            | Parts |
|--------------------------------------------|-------|
| Chromocitronine R (colour index No. 441)   | 3     |
| Urea                                       | 3     |
| $\omega:\omega'$ -dihydroxydiethylsulphide | 3     |
| Hot water                                  | 24.9  |
| Tragacanth thickening                      | 50    |
| Ammonium sulphocyanate, solution 1:1       | 3     |
| Sodium chromate, solution 1:2              | 6     |
| Sodium thiosulphate, solution 1:1          | 6     |
| Ammonia                                    | 1     |
| Hydroquinone                               | 0.1   |
|                                            | 100   |

The printed material is dried, left lying or hanging at room temperature for 48 hours, then rinsed, soaped at 60° C., rinsed and dried.

Thus deep and even yellow prints are obtained.

The printed material is dried, left lying for 48 hours, rinsed, soaped at 60° C., rinsed and dried. Thus a deep, even, green print is obtained.

which are as strong as the prints obtained with chromium acetate by a steaming for 1 hour.

#### Example 2

The following printing paste is printed on cotton:

|                                                                        | Parts |
|------------------------------------------------------------------------|-------|
| Dyestuff obtained according to Example 1 of British Patent No. 255,086 | 3     |
| Urea                                                                   | 3     |
| $\omega:\omega'$ -dihydroxydiethylsulphide                             | 3     |
| Hot water                                                              | 24.8  |
| Tragacanth thickening                                                  | 50    |
| Ammonium sulphocyanate, solution 1:1                                   | 3     |
| Sodium chromate, solution 1:2                                          | 6     |
| Sodium thiosulphate, solution 1:1                                      | 6     |
| Ammonia                                                                | 1     |
| $\alpha$ -naphthoquinone                                               | 0.2   |
|                                                                        | 100   |

The printed material is dried and steamed for 2 minutes, then rinsed and soaped at 60° C., rinsed and dried.

Thus deep, vivid, orange prints are obtained, which are as deep and vivid as the prints obtained with chromium acetate and by a steaming for 1 hour.

#### Example 3

The following printing colour is printed on cotton or viscose-rayon:

|                                                                           | Parts |
|---------------------------------------------------------------------------|-------|
| Dyestuff prepared according to Example 1 of the French Patent No. 457,840 | 3     |
| Urea                                                                      | 3     |
| $\omega:\omega'$ -dihydroxydiethylsulphide                                | 5     |
| Hot water                                                                 | 22.1  |
| Tragacanth thickening                                                     | 50    |
| Ammonium sulphate, solution 1:2                                           | 4     |
| Ammonium chromate, solution 1:2                                           | 5.5   |
| Sodium thiosulphate, solution 1:1                                         | 6     |
| Ammonia                                                                   | 1     |
| Anthraquinone                                                             | 0.4   |
|                                                                           | 100   |

The printed material is dried and steamed for 2 minutes, then rinsed, soaped at 60° C., rinsed and dried. Thus deep, even, vivid, yellowish-red prints are obtained, which are rather stronger than prints obtained with chromium acetate by a steaming of 60 minutes.

#### Example 4

The following printing colour is printed on cotton:

|                                                                            | Parts |
|----------------------------------------------------------------------------|-------|
| Dyestuff obtained according to Example 1 of the British Patent No. 500,075 | 3     |
| Urea                                                                       | 3     |
| $\omega:\omega'$ -dihydroxydiethylsulphide                                 | 5     |
| Hot water                                                                  | 26.8  |
| Tragacanth thickening                                                      | 50    |
| Ammonium chloride, solution 1:1                                            | 3     |
| Ammonium chromate cryst.                                                   | 1.8   |
| Ammonia                                                                    | 1     |
| Sodium thiosulphate, solution 1:1                                          | 6     |
| Anthraquinone                                                              | 0.4   |
|                                                                            | 100   |

The printed material is dried, left lying for 48 hours, rinsed, soaped at 60° C., rinsed and dried. Thus a deep, even, green print is obtained.

## 5

## Example 5

|                                                                        | Parts |
|------------------------------------------------------------------------|-------|
| Portion A:                                                             |       |
| Dyestuff obtained according to Example 2 of the British Patent 231,885 | 3     |
| Urea                                                                   | 3     |
| $\omega:\omega'$ -dihydroxydiethylsulphide                             | 5     |
| Hot water                                                              | 11    |
| Tragacanth thickening                                                  | 25    |
| Ammonium sulphate, solution 1:2                                        | 4     |
| Sodium thiosulphate, solution 1:1                                      | 6     |
|                                                                        | 57    |
| Portion B:                                                             |       |
| Water                                                                  | 10.8  |
| Tragacanth thickening                                                  | 25    |
| Ammonium bichromate, solution 1:1                                      | 6     |
| Ammonia                                                                | 1     |
| Anthraquinone                                                          | 0.2   |
|                                                                        | 43    |

Portion A and Portion B are mixed before use. With the paste thus obtained cotton or viscose-rayon is printed. The printed material is dried, allowed to lie for 48 hours, rinsed, soaped at 60° C., rinsed and dried. There are obtained deep, even, red prints.

## Example 6

The following printing colour is printed on cotton:

|                                            | Parts |
|--------------------------------------------|-------|
| Chromocitronine 3 R (colour index No. 441) | 3     |
| Urea                                       | 3     |
| $\omega:\omega'$ -dihydroxydiethylsulphide | 3     |
| Hot water                                  | 23.9  |
| Tragacanth thickening                      | 50    |
| Ammonium sulphate, solution 1:2            | 4     |
| Sodium chromate, solution 1:2              | 6     |
| Ammonium sulphite, solution 1:1            | 6     |
| Ammonia                                    | 1     |
| Hydroquinone                               | 0.1   |
|                                            | 100   |

The printed material is dried, left lying for 48 hours, rinsed, soaped at 60° C., rinsed and dried.

Thus deep yellow prints are obtained.

## Example 7

The following printing paste is prepared:

|                                            | Parts |
|--------------------------------------------|-------|
| Chromocitronine R (colour index No. 441)   | 3     |
| Acetamide                                  | 3     |
| $\omega:\omega'$ -dihydroxydiethylsulphide | 5     |
| Water                                      | 22.9  |
| Tragacanth thickening                      | 50    |
| Ammonium sulphocyanate, solution 1:1       | 3     |
| Sodium chromate, solution 1:2              | 6     |
| Sodium thiosulphate, solution 1:1          | 6     |
| Ammonia                                    | 1     |
| Resorcinol                                 | 0.1   |
|                                            | 100   |

The printed material is dried, left lying for 48 hours, rinsed, soaped at 60° C., rinsed and dried.

Thus deep, even, yellow prints are obtained.

The quantity of resorcinol used in this example may be replaced by 0.2 part of pyrogallic sulphonic acid, the results being not modified in any way.

## 6

## Example 8

The following printing paste is prepared:

|                                            | Parts |
|--------------------------------------------|-------|
| Blue 1900 double (colour index No. 892)    | 3     |
| Formic acid 85%                            | 2     |
| Urea                                       | 3     |
| $\omega:\omega'$ -dihydroxydiethylsulphide | 3     |
| Hot water                                  | 27.5  |
| Tragacanth thickening                      | 50    |

Dissolve, cool down and add:

|                               |     |
|-------------------------------|-----|
| Sodium hydrosulphite powder   | 4   |
| Ammonium nitrate cryst.       | 4   |
| Sodium chromate, solution 1:2 | 1.5 |
| Formic acid 85%               | 2   |
|                               | 100 |

20 The printed cellulose material is dried and left lying for 48 hours, rinsed, soaped at 60° C., rinsed and dried.

Thus vivid, deep, reddish-blue prints are obtained, which are as deep as the blue prints obtained with the same quantity of dyestuff and with chromium acetate by a steaming of 60 minutes.

## Example 9

30 The following printing colour is printed on viscose rayon, staple fibre or cotton:

|                                                                              | Parts |
|------------------------------------------------------------------------------|-------|
| Dyestuff obtained according to Example 2 of the British Patent No. 3796/1914 | 3     |
| 35 Urea                                                                      | 3     |
| Hot water                                                                    | 28    |
| Tragacanth thickening                                                        | 50    |
| Ammonium sulphocyanate, solution 1:1                                         | 3     |
| 40 Sodium chromate, solution 1:2                                             | 6     |
| Sodium thiosulphate, solution 1:1                                            | 6     |
| Ammonia                                                                      | 1     |
|                                                                              | 100   |

45 The printed material is dried, steamed for 2 minutes in the Mather-Platt ager, washed, soaped at 60° C. and finished.

Thus there are obtained vivid, deep pink prints, which are at least as strong as the pink prints obtainable with the same quantity of dyestuff and with chromium acetate by a steaming for 1 hour.

## Example 10

55 The following printing paste is printed on cotton, viscose rayon or staple fibre:

|                                         | Parts |
|-----------------------------------------|-------|
| Chromorhodine BB (colour index No. 762) | 3     |
| Urea                                    | 3     |
| 60 Hot water                            | 27.5  |
| Tragacanth thickening                   | 50    |
| Ammonium sulphate, solution 1:2         | 4     |
| Ammonium chromate, solution 1:2         | 5.5   |
| Sodium thiosulphate, solution 1:1       | 6     |
| 65 Ammonia                              | 1     |
|                                         | 100   |

70 The printed material is dried, steamed for 2 minutes, rinsed, soaped at 60° C., rinsed and dried.

Thus there are obtained vivid, deep pink prints which are at least as strong as the prints obtained with the same quantity of dyestuff and with chromium acetate by a steaming for 60 minutes.

7  
Example 11

The following printing colour is printed on cotton:

|                                                                            | Parts |
|----------------------------------------------------------------------------|-------|
| Dyestuff obtained according to Example 1 of the British Patent No. 255,086 | 3     |
| Urea                                                                       | 3     |
| $\omega:\omega'$ -dihydroxydiethylsulphide                                 | 5     |
| Hot water                                                                  | 22.6  |
| Tragacanth thickening                                                      | 50    |
| Ammonium sulphate, solution 1:2                                            | 4     |
| Sodium chromate, solution 1:2                                              | 6     |
| Sodium thiosulphate, solution 1:1                                          | 6     |
| Anthraquinone powder                                                       | 0.4   |
|                                                                            | 100   |

The printed material is dried, left lying for 48 hours, rinsed, soaped at 50° C., rinsed again and finished.

Thus vivid, deep, orange prints are obtained, which are as strong as the prints obtained with chromium acetate by a steaming duration of 1 hour.

## Example 12

The following printing colour is printed on cotton:

|                                                                        | Parts |
|------------------------------------------------------------------------|-------|
| Dyestuff prepared according to Example 1 of the British Patent 500,075 | 3     |
| Urea                                                                   | 3     |
| $\omega:\omega'$ -dihydroxydiethylsulphide                             | 5     |
| Hot water                                                              | 21.6  |
| Tragacanth thickening                                                  | 50    |
| Ammonium sulphate, solution 1:2                                        | 4     |
| Sodium chromate, solution 1:2                                          | 6     |
| Ammonia                                                                | 1     |
| Sodium thiosulphate, solution 1:1                                      | 6     |
| Anthraquinone                                                          | 0.4   |
|                                                                        | 100   |

The printed material is dried, left lying for 48 hours, rinsed, soaped at 50° C., rinsed again and finished.

Thus deep, vivid green prints are obtained, which are as strong as the green prints obtained with the same quantity of dyestuff and with chromium acetate by a steaming for 60 minutes.

## Example 13

The following printing paste is printed on cotton:

|                                                | Parts |
|------------------------------------------------|-------|
| Chrome violet CB double (colour index No. 727) | 3     |
| Urea                                           | 3     |
| $\omega:\omega'$ -dihydroxydiethylsulphide     | 5     |
| Hot water                                      | 22.1  |
| Tragacanth thickening                          | 50    |
| Ammonium sulphate, solution 1:2                | 4     |
| Ammonium chromate, solution 1:2                | 5.5   |
| Ammonia                                        | 1     |
| Sodium thiosulphate, solution 1:1              | 6     |
| Anthraquinone                                  | 0.4   |
|                                                | 100   |

The printed material is dried, left lying for 48 hours or steamed during 2 minutes, rinsed, soaped at 50° C., rinsed again and finished.

Thus there are obtained deep, vivid, violet prints, which are at least as strong as the violet prints obtained with the same quantity of dyestuff and with chromium acetate by a steaming for 60 minutes.

## Example 14

|                                                                             | Parts |
|-----------------------------------------------------------------------------|-------|
| Dyestuff obtained according to the example of the French Patent No. 398,980 | 3     |
| Urea                                                                        | 3     |
| $\omega:\omega'$ -dihydroxydiethylsulphide                                  | 5     |
| Water                                                                       | 25.8  |
| Tragacanth thickening                                                       | 50    |
| Ammonium sulphate, solution 1:2                                             | 4     |
| Ammonium chromate cryst.                                                    | 1.8   |
| Sodium thiosulphate, solution 1:1                                           | 6     |
| Ammonia                                                                     | 1     |
| Anthraquinone powder                                                        | 0.4   |
|                                                                             | 100   |

The printed material is dried, left lying for 48 hours, rinsed, soaped at 50° C., rinsed again and dried.

Thus there are obtained deep, even orange prints corresponding in every respect to the orange prints obtainable with chromium acetate by a steaming for 60 minutes.

| 25 | Examples                                                                    | 15    | 16    | 17    | 18    |
|----|-----------------------------------------------------------------------------|-------|-------|-------|-------|
|    |                                                                             | Parts | Parts | Parts | Parts |
|    | The following printing pastes are printed on wall-paper:                    |       |       |       |       |
|    | Dyestuff obtained according to Example 2 of the British Patent No. 3,796/14 | 0.8   |       |       |       |
|    | Dyestuff obtained according to Example 1 of the British Patent No. 500,075  |       | 0.8   |       |       |
|    | Dyestuff obtained according to Example 1 of the British Patent No. 255,086  |       |       | 0.8   |       |
|    | Chromocitrone R (Colour Index No. 441)                                      |       |       |       | 0.8   |
|    | Urea                                                                        | 3     | 3     | 3     | 3     |
|    | $\omega:\omega'$ -dihydroxydiethylsulphide                                  | 3     | 3     | 3     | 3     |
|    | Water                                                                       | 10    | 10    | 11    | 10    |
|    | Tragacanth thickening                                                       | 70    | 70    | 70    | 70    |
|    | Ammonium sulphate, solution 1:2                                             | 4     | 4     | 4     | 4     |
|    | Ammonium chromate cryst.                                                    | 1.8   | 1.8   | 1.8   | 1.8   |
|    | Sodium thiosulphate, solution 1:1                                           | 6     | 6     | 6     | 6     |
|    | Anthraquinone powder                                                        | 0.4   | 0.4   | 0.4   | 0.4   |
|    | Ammonia                                                                     | 1     | 1     |       | 1     |
|    |                                                                             | 100   | 100   | 100   | 100   |

The printed wall paper is dried on drying drums and hung up for 48 hours.

Thus deep, bright and well fixed prints are obtained, which according to Example 15 are pink, and according to Example 16 green, while according to Example 17 they are brownish orange and according to Example 18 yellow.

All the prints are fast to rubbing and the printed paper-hangings may be washed without damage.

What I claim is:

1. A process for printing cellulosic material with chrome dyestuffs, which comprises printing onto the said cellulosic material a printing paste containing, besides the dyestuff, a thickener, a water-soluble carboxylic acid amide, as chromium mordant an alkali metal chromate, a substance which splits off a strong acid in the heat and, as characteristic additions, a water-soluble salt of an inorganic acid derived from an oxygen compound of sulphur and possessing reducing properties, an aromatic compound capable of performing the reversible reaction quinone  $\leftrightarrow$  hydroquinone, and  $\omega:\omega'$ -dihydroxydiethyl sulphide, and subjecting the obtained prints to a drying operation.

2. A process for printing cellulosic material with chrome mordant dyestuffs, which comprises printing onto the said cellulosic material a printing paste containing, besides the dyestuff, a

thickener, a water-soluble carboxylic acid amide, as chromium mordant an alkali metal chromate, a substance which splits off a strong acid in the heat and, as characteristic additions, a water-soluble salt of an inorganic acid derived from an oxygen compound of sulphur and possessing reducing properties, an aromatic compound capable of performing the reversible reaction quinone  $\leftrightarrow$  hydroquinone, and  $\omega:\omega'$ -dihydroxydiethyl sulphide, and subjecting the obtained prints to a drying operation and steaming for 2 minutes.

3. A process for printing cellulosic material with chrome mordant dyestuffs, which comprises printing onto the said cellulosic material a printing paste containing, besides the dyestuff, a thickener, urea, as chromium mordant an alkali metal chromate, a substance which splits off a strong acid in the heat and, as characteristic additions, a water-soluble salt of an inorganic acid derived from an oxygen compound of sulphur and possessing reducing properties, an aromatic compound capable of performing the reversible reaction quinone  $\leftrightarrow$  hydroquinone, and  $\omega:\omega'$ -dihydroxydiethyl sulphide, and suspending the printed cellulosic material until dry.

4. A process for printing cellulosic material with chrome mordant dyestuffs, which comprises printing onto the said cellulosic material a printing paste containing, besides the dyestuff, a thickener, a water-soluble carboxylic acid amide, as chromium mordant sodium chromate, a substance which splits off a strong acid in the heat and, as characteristic additions, a water-soluble salt of an inorganic acid derived from an oxygen compound of sulphur and possessing reducing properties, an aromatic compound capable of performing the reversible reaction quinone  $\leftrightarrow$  hydroquinone, and  $\omega:\omega'$ -dihydroxydiethyl sulphide, and suspending the printed cellulosic material until dry.

5. A process for printing cellulosic material with chrome mordant dyestuffs, which comprises printing onto the said cellulosic material a printing paste containing, besides the dyestuff, a thickener, a water-soluble carboxylic acid amide, as chromium mordant an alkali metal chromate, ammonium sulphate and, as characteristic additions, a water-soluble salt of an inorganic acid derived from an oxygen compound of sulphur and possessing reducing properties, an aromatic compound capable of performing the reversible reaction quinone  $\leftrightarrow$  hydroquinone, and  $\omega:\omega'$ -dihydroxydiethyl sulphide, and suspending the printed cellulosic material until dry.

6. A process for printing cellulosic material with chrome mordant dyestuffs, which comprises printing onto the said cellulosic material a printing paste containing, besides the dyestuff, a thickener, a water-soluble carboxylic acid amide, as chromium mordant an alkali metal chromate, a substance which splits off a strong acid in the heat and, as characteristic additions, sodium thiosulphate, an aromatic compound capable of performing the reversible reaction quinone  $\leftrightarrow$  hydroquinone, and  $\omega:\omega'$ -dihydroxydiethyl sulphide, and suspending the printed cellulose material until dry.

7. A process for printing cellulosic material with chrome mordant dyestuffs, which comprises printing onto the said cellulosic material a printing paste containing, besides the dyestuff, a thickener, a water-soluble carboxylic acid amide, as chromium mordant an alkali metal chromate, a substance which splits off a strong acid in the heat and, as characteristic additions, a water-

soluble salt of an inorganic acid derived from an oxygen compound of sulphur and possessing reducing properties, anthraquinone and  $\omega:\omega'$ -dihydroxydiethyl sulphide, and suspending the printed material until dry.

8. A process for printing cellulose material with chrome mordant dyestuffs, which comprises printing onto the said cellulosic material a printing paste containing, besides the dyestuff, a thickener, a water-soluble carboxylic acid amide, as chromium mordant an alkali metal chromate, a substance which splits off a strong acid in the heat and, as characteristic additions, a water-soluble salt of an inorganic acid derived from an oxygen compound of sulphur and possessing reducing properties, hydroquinone and  $\omega:\omega'$ -dihydroxydiethyl sulphide, and suspending the printed cellulosic material until dry.

9. A process for printing cotton with chrome mordant dyestuffs, which comprises printing onto the cotton a printing paste containing, besides the dyestuff, a thickener, a water-soluble carboxylic acid amide, as chromium mordant an alkali metal chromate, a substance which splits off a strong acid in the heat and, as characteristic additions, a water-soluble salt of an inorganic acid derived from an oxygen compound of sulphur and possessing reducing properties, an aromatic compound capable of performing the reversible reaction quinone  $\leftrightarrow$  hydroquinone and  $\omega:\omega'$ -dihydroxydiethyl sulphide, and suspending the printed cotton until dry.

10. A process for printing paper-hangings with chrome mordant dyestuffs, which comprises printing onto the paper-hangings a printing paste containing, besides the dyestuff, a thickener, a water-soluble carboxylic acid amide, as chromium mordant an alkali metal chromate, a substance which splits off a strong acid in the heat and, as characteristic additions, a water-soluble salt of an inorganic acid derived from an oxygen compound of sulphur and possessing reducing properties, an aromatic compound capable of performing the reversible reaction quinone  $\leftrightarrow$  hydroquinone, and  $\omega:\omega'$ -dihydroxydiethyl sulphide, and subjecting the obtained prints to a drying operation and hanging the same.

11. A printing paste containing beside a chrome mordant a dyestuff, a thickener, a water-soluble carboxylic acid amide, as chromium mordant, an alkali metal chromate, a substance which splits off a strong acid in the heat and, as characteristic additions, a water-soluble salt of an inorganic acid derived from an oxygen compound of sulphur and possessing reducing properties, an aromatic compound capable of performing the reversible reaction quinone  $\leftrightarrow$  hydroquinone, and  $\omega:\omega'$ -dihydroxydiethyl sulphide.

12. A printing paste containing beside a chrome mordant dyestuff, a thickener, a water-soluble carboxylic acid amide, as chromium mordant, an alkali metal chromate, a substance which splits off a strong acid in the heat and, as characteristic additions, sodium thiosulphate, an aromatic compound capable of performing the reversible reaction quinone  $\leftrightarrow$  hydroquinone, and  $\omega:\omega'$ -dihydroxydiethyl sulphide.

13. A printing paste containing beside a chrome mordant dyestuff, a thickener, a water-soluble carboxylic acid amide, as chromium mordant, an alkali metal chromate, a substance which splits off a strong acid in the heat and, as characteristic additions, a water-soluble salt

of an inorganic acid derived from an oxygen compound of sulphur and possessing reducing properties, anthraquinone, and  $\omega : \omega'$ -dihydroxyethyl sulphide.

14. A printing paste containing beside a chrome mordant dyestuff, a thickener, a water-soluble carboxylic acid amide, as chromium mordant, an alkali metal chromate, a substance which splits off a strong acid in the heat and, as characteristic additions, a water-soluble salt of an inorganic acid derived from an oxygen compound of sulphur and possessing reducing properties, hydroquinone, and  $\omega : \omega'$ -dihydroxydiethyl sulphide.

15. ERNST TSCHAN.

#### REFERENCES CITED

The following references are of record in the file of this patent:

#### UNITED STATES PATENTS

| Number    | Name   | Date           |
|-----------|--------|----------------|
| 1,942,774 | Roulet | Jan. 9, 1934   |
| 2,018,436 | Brandt | Oct. 22, 1935  |
| 2,131,320 | Gubler | Sept. 27, 1938 |

#### FOREIGN PATENTS

| Number  | Country | Date          |
|---------|---------|---------------|
| 203,131 | Germany | Oct. 15, 1908 |